

Dec. 4, 1956

G. H. LACY

2,772,994

LAMINATED THREAD

Filed Oct. 18, 1954

2 Sheets-Sheet 1



FIG. 1

FIG. 2



FIG. 3

INVENTOR.

GEORGE H. LACY

BY *Ely, Pearne & Gordon*

ATTORNEYS

Dec. 4, 1956

G. H. LACY  
LAMINATED THREAD

2,772,994

Filed Oct. 18, 1954

2 Sheets-Sheet 2



INVENTOR.  
GEORGE H. LACY  
BY *Ely, Pearne & Gordon*  
ATTORNEYS

# United States Patent Office

2,772,994

Patented Dec. 4, 1956

1

2,772,994

## LAMINATED THREAD

George H. Lacy, Cleveland, Ohio, assignor to The Dobeck-mun Company, Cleveland, Ohio, a corporation of Ohio

Application October 18, 1954, Serial No. 462,753

12 Claims. (Cl. 154—53.6)

This invention relates to fabric manufacture and to threads to be used in such manufacture. More particularly, the invention pertains to multicolor threads and fabrics.

This application is a continuation-in-part with respect to application Serial No. 400,653 filed December 28, 1953, now abandoned.

An object of the invention is to provide a means of manufacturing fabrics or textiles with predetermined patterns or effects of various types, while employing weaving procedures no more complex than those required to weave conventional solid-color fabrics.

Another object of the invention is to provide pattern effects and multicolored textile effects which have heretofore not been attainable or which have been attainable only through the use of very costly procedures and equipment, but which may be inexpensively provided in accordance with the present invention.

Another object of the invention is to provide a thread which may be employed in the simplest type of conventional weaving operations to provide finish effects which have heretofore been relatively costly and difficult to produce, many such effects involving the use of costly specialized textile machinery or special procedures. Thus, the threads to which the present invention relates may be employed with the most simple types of weaving equipment to produce moire effects, boucle effects and "shot-through" or flecked effects, gimping effects and others.

The above and other objects and advantages of the invention will become clear from the following specification of certain embodiments of the invention, together with the drawings in which:

Figures 1 and 2 comprise a schematic representation of one method of producing threads according to the present invention;

Figure 3 is a view on a scale greatly enlarged from that of Figure 1 showing a thread produced according to the present invention;

Figure 4 is a view on an intermediate scale showing a web from which threads are to be formed;

Figure 5 is a view similar to Figure 3 showing another thread produced according to the invention;

Figure 6 is a view similar to Figure 4, showing another web from which threads are to be formed;

Figure 7 is a view similar to Figures 4 and 6 showing still another web from which threads are to be formed.

Thread contemplated by the invention may comprise laminations of strips of transparent or semi-transparent material with metal foil or metallic deposits included therein. One material which may be employed is cellulose acetate butyrate, although strips of other cellulosic materials, preferably containing suitable plasticizers, may be used (e. g., cellulose acetate, cellulose acetate propionate). Other non-cellulosic material may also be employed, as for example, longitudinally and transversely oriented films of polymerized ethylene glycol terephthalate.

2

In accordance with the present invention, thread is preferably formed by providing sheets of the material from which the thread is to be made, printing such sheets with transversely extending bands of color or patterns, preferably having sharply defined boundaries, and slitting the sheets lengthwise to provide a number of individual threads. Several sheets may be combined or laminated together prior to slitting in order to provide threads having several thicknesses, and color or pattern applied to one or all of said sheets is preferably included within such lamination rather than being exposed on one or both of the outer surfaces of the lamination. Sheeted material may be combined with metal foil, such as aluminum foil, or may receive a metal vapor deposit (as disclosed in copending application of Karl E. Prindle and George Lacy, Serial No. 267,108, filed January 18, 1952, now Patent No. 2,714,569) in order to provide threads having a metallic appearance, printing of the patterns or bands of color occurring either before or after or both before and after the foil combining or metal depositing operation. The film of metal foil or the deposited metal film may itself be printed, if desired. (As used in this specification and in the appended claims, the term "film" is understood to include foil or metal vapor deposits or other metal layers.) Numerous transparent adhesives which are suitable for the lamination of webs of the various materials from which the thread contemplated by the invention may be formed will be apparent to those skilled in the art. Such adhesives may be adapted to pigmentation so that the adhesives themselves may exhibit a color, if desired. Thus, the pigmented adhesives specified in the above-mentioned application, Serial No. 267,108, may be employed, if desired. Obviously, the same adhesive formulations as set forth in such application, minus the pigments set forth therein, may be employed if a colorless adhesive is desired. By way of example, the following formulations for suitable transparent adhesives are given or are again set forth as follows on the basis of 100 pound lots:

### Example 1

|                             | Pounds |
|-----------------------------|--------|
| Coconut oil alkyd resin     | 16.4   |
| R. S.—½ sec. nitrocellulose | 9.7    |
| Textile spirits             | 30.6   |
| Isopropyl acetate           | 34.2   |
| Tricresyl phosphate         | 9.1    |
|                             | 100.0  |

### Example 2

|                         | Pounds |
|-------------------------|--------|
| Polyvinyl acetate resin | 20.4   |
| Tricresyl phosphate     | 10.2   |
| Toluol                  | 40.7   |
| Isopropyl acetate       | 28.7   |
|                         | 100.0  |

### Example 3

|                                     | Pounds |
|-------------------------------------|--------|
| Acrylonitrile-butadiene copolymer   | 7.5    |
| Vinyl acetate-chloride copolymer    | 1.5    |
| Aryl sulfonamide-formaldehyde resin | 8.0    |
| Toluol                              | 60.0   |
| Methylethyl ketone                  | 23.0   |
|                                     | 100.0  |

The thread may be produced as shown schematically in Figures 1 and 2. Here, the webs 10 and 11 of the preferably transparent web material are supplied by the feed rolls 12 and 13. In the particular embodiment illustrated in Figures 1 and 2, a metal foil 15 supplied from the feed roll 16 is laminated between the webs 10

and 11 by the laminating rolls 17. The webs 10 and 11 are printed with a striped pattern by the printing rolls 14. The patterns on both webs are preferably registered with each other by positioning the webs so that the patterns on the respective webs directly overlie each other in the bight between the laminating rolls. The pattern may comprise unprinted or clear stripes 18 which, in the laminated form, reveal the metallic surface of the foil 15. The colored portions 19 may be opaque or partially transparent or translucent, depending on the particular ink or color employed and may partially or totally obscure the metallic surface of the foil 15. The lamination may be taken up on the roll 22. As shown in Figure 2, the laminated web is then slit into numerous threads 20 by suitable means such as the knives 21, the threads preferably being taken up on spools (not shown). If desired, the slitting may be performed in two stages—the laminated web being first slit into relatively broad bands which are taken up on rolls, each of which is then fed through a bank of knives similar to the knives 21 schematically illustrated in Figure 2. In such a procedure, the cutting knives need only extend across the width of a band rather than the width of the entire web.

A thread produced as described above is illustrated in Figure 3. The thread presents clearly delineated areas of different colors which may be sharply contrasted. The thread may then be employed in woven patterns, either as a warp or filler, and may be woven twisted or flat. Particularly when twisted and employed on a background of fairly solid color, the thread has the appearance and rich effect of gimping, the intermittently visible metal appearing to be interlaced as part of a gimped strip or design.

It will be apparent that the web from which the threads are cut may be printed in two or three or more different colors and that each color may be printed so that it extends a short distance or a considerable distance along the resulting threads. The metal foil or vapor deposit may be covered with a transparent ink which may have a metallic color, or a colored adhesive may be employed to adhere the laminants in order to give the metallic foil any metallic color desired. For example, the aluminum foil which has a silver appearance may be given the appearance of gold by using a suitable yellow ink or laminant adhesive (as disclosed in the above mentioned application, Serial No. 267,108).

Accordingly, threads produced by the invention may have multicolored stripes or patterns of any desired conformation and arrangement; the colors may be metallic or non-metallic. The stripe or pattern may be consistent for a given thread production, or it may be varied as set forth below.

One effect which is frequently desired in fabrics, particularly when metallic colors are employed, is a random "shot-through" or flecked effect. In this connection, a patterned lamination such as that illustrated in Figure 4 may be provided according to the procedures described above. Here the metal foil is exposed at relatively narrow clear areas or stripes 23 which are irregularly spaced in a field of solid color 24. Threads slit from this pattern will have an appearance similar to the thread illustrated in Figure 5. The solid color 24 is chosen to match or approximate the background color of the fabric in which the thread is to be employed. The finished fabric will exhibit what appear to be arbitrarily spaced metallic flecks in a solid background.

If the flecked effect is to be relatively dense or intense, it may be desirable to provide threads having patterns which vary from thread to thread in order to avoid any regularity in the final pattern. In Figure 6, a lamination is illustrated similar to that shown in Figure 4, except that the clear stripes 25 are non-parallel. It will be apparent that each of the threads cut from the web illustrated in Figure 6 will have a pattern different from the other threads cut from the same web. Even in a dense

pattern of such threads, no regularity or striation will occur.

It is not necessary for the printing on the web to be in the form of stripes or bars, as in the preceding examples.

5 The pattern may be in the form of any type of design, as the box design on the web 27 shown in Figure 7. And, while the pre-printing of webs from which threads are to be formed has been described above in connection with what may be termed heavy or massive designs or patterns, 10 it will be apparent that fine dotted or lined patterns may be employed in pre-printing the thread. For example, Benday type prints may be employed on the unslit web to provide an apparent gradual shading from one color to another along the length of the threads.

15 It is to be observed that the pre-printed threads to which this invention relates may be employed as a warp or filler or both.

The many possible alternatives in the invention which are described above will make it apparent that the scope 20 of the invention is not limited to the details of specifically illustrated embodiments. The scope of the invention is defined in the following claims.

What is claimed is:

1. A thread comprising a metal film interposed between 25 laminated long narrow strips of transparent thermoplastic, and at least one printed color deposit of a given color intermittently overlying said metal film along the length of said long narrow strips, said at least one color deposit being covered by at least one of said narrow strips.

30 2. A thread comprising an aluminum film interposed between laminated long narrow strips of cellulose acetate butyrate, and at least one printed color deposit of a given color intermittently overlying said aluminum film along the length of said long narrow strips, said at least one color deposit being covered by at least one of said narrow strips.

35 3. A thread comprising an aluminum film interposed between laminated long narrow strips of transparent non-fibrous cellulosic material, and at least one printed color 40 deposit of a given color intermittently overlying said aluminum film along the length of said long narrow strips, said at least one color deposit being covered by at least one of said narrow strips.

45 4. A thread comprising an aluminum film interposed between laminated long narrow strips of polymerized ethylene glycol terephthalate, and at least one printed color deposit of a given color intermittently overlying said aluminum film along the length of said long narrow strips, said at least one color deposit being covered by at least one of said narrow strips.

50 5. A thread comprising a metal film interposed between a pair of laminated long narrow strips of transparent thermoplastic, at least one printed color deposit 55 of a given color on the inner side of at least one of said strips and covered by said thermoplastic and intermittently overlying said metal film along the length of said long narrow strips.

60 6. A thread comprising a metal film interposed between a pair of laminated long narrow strips of transparent thermoplastic, at least one printed color deposit 65 of a given color on the inner side of each of said strips and covered by said thermoplastic and intermittently overlying said metal film along the length of said long narrow strips.

65 7. A thread comprising a metal film included within a lamination of at least two long narrow strips of transparent thermoplastic, at least one printed color deposit of a given color intermittently overlying each side of 70 said metal film along the length of said long narrow strips, said at least one color deposit on each side of said metal being covered by at least one of said narrow strips.

75 8. A thread comprising a metal film included within a lamination of at least two long narrow strips of transparent thermoplastic, a plurality of printed color deposits of given colors intermittently overlying said metal film

along the length of said long narrow strips, said color deposits being covered by at least one of said narrow strips.

9. A thread comprising a metal film included within a lamination of at least two long narrow strips of transparent thermoplastic, a color deposit of a given color intermittently overlying each side of said metal film along the length of said long narrow strips, said color deposit on each side of said metal film being covered by at least one of said narrow strips.

10. A thread comprising a metal film included within a lamination of at least two long narrow strips of transparent thermoplastic, a plurality of printed color deposits of given colors intermittently overlying one side of said metal film along the length of said long narrow strips, and a plurality of printed color deposits of given colors intermittently overlying the other side of said metal film along the length of said long narrow strips, each of said color deposits being covered by at least one of said long narrow strips.

11. A thread comprising a metal film included within a lamination of at least two long narrow strips of transparent thermoplastic, and at least one printed color de-

15  
10

posit of a given color intermittently overlying said metal film along the length of said long narrow strips, said at least one color deposit being covered by at least one of said narrow strips.

12. A thread comprising a metal film interposed between laminated long narrow strips of transparent non-fibrous cellulosic material and at least one printed color deposit of a given color intermittently overlying said metal film along the length of said long narrow strips, said at least one color deposit being covered by at least one of said narrow strips.

## References Cited in the file of this patent

## UNITED STATES PATENTS

|           |                |                |
|-----------|----------------|----------------|
| 1,651,649 | Waite          | Dec. 6, 1927   |
| 1,913,397 | Knecht         | June 13, 1933  |
| 2,118,847 | Katz           | May 31, 1938   |
| 2,129,504 | Prindle        | Sept. 6, 1938  |
| 2,482,981 | Kamrass        | Sept. 27, 1949 |
| 2,569,764 | Jonas          | Oct. 2, 1951   |
| 2,607,185 | Silverman      | Aug. 19, 1952  |
| 2,714,569 | Prindle et al. | Aug. 2, 1955   |